

# United States Patent [19]

Turner

[11] 3,830,023

[45] Aug. 20, 1974

[54] DRY DESCALING

[75] Inventor: Charles A. Turner, Flourtown, Pa.

[73] Assignee: Selas Corporation of America,  
Dresher, Pa.

[22] Filed: Oct. 30, 1972

[21] Appl. No.: 302,067

[52] U.S. Cl. .... 51/322

[51] Int. Cl. .... B24b 1/00

[58] Field of Search..... 51/322, 323, 324

[56] References Cited

UNITED STATES PATENTS

3,166,841 1/1965 Gebhard ..... 51/322 UX

3,699,726 10/1972 Turner ..... 51/322

Primary Examiner—Donald G. Kelly

[57] ABSTRACT

Dry descaling of hot-rolled, steel strip wherein the strip, having a layer of magnetite on its surface, is heated in a normal furnace atmosphere to at least 1,500°F such that conversion of the magnetite to wustite is effected. Thereafter, the strip is immediately quenched below 600°F by air jets at a rate rapid enough to prevent reconversion of the wustite to magnetite. The wustite scale is subsequently removed by abrasion.

3 Claims, No Drawings

## DRY DESCALING

The present invention relates to the descaling of steel and more particularly to a method of dry descaling of strip metal utilizing heat conversion of the scale followed by a mechanical removal means.

In the manufacture of hot-rolled strip steel, the metal, as it leaves the hot rolls is coiled either just below the rolling temperature or at a lower temperature. In either case, a scale in the form of magnetite results on the surface. This scale must be removed before the strip is used in the hot-rolled condition or is cold reduced to lighter gauges. Various methods of removing the scale are practiced, the most usual of which is acid pickling. Another method of scale removal is described in the Patent to Gebhard et al., No. 3,166,841, in which the hot-rolled strip is heated in an inert atmosphere to a temperature above 1076°F. At this temperature magnetite converts to wustite, a more easily removed scale. The strip must then be cooled under an inert atmosphere to below the reconversion temperature before the wustite scale is removed by pickling or mechanical action.

Another dry descaling method is disclosed in Turner et al., Patent No. 3,699,726, in which the hot-rolled strip is heated in the atmosphere to not above the  $A_{C_1}$  transformation temperature or 1400°F maximum, but above 1076°F, to convert the magnetite to wustite. The strip is then rapidly cooled below 600°F by air jets before being run through breaker rolls and subjected to abrasive action to remove the scale. This process while being fairly simple and producing a clean strip has the disadvantage of hardening the strip. The breaker rolls induce a strain that results in subsequent spontaneous age hardening of several points. While for some end uses this is of no consequence, for other uses, such as deep drawing, the increased hardness is objectionable.

The Gebhard patent and the Turner et al. patents are based upon consideration of converting the prior scale, as magnetite, to wustite. Aside from satisfying this basic purpose, it has been established that sub-critical heating for scale conversion accounts for a substantial hardening effect on the steel strip, amounting to an increase of Rockwell B hardness of some 15 to 20 points. This hardening results from an alteration in the iron carbide size and distribution by the heating to a sub-critical temperature with subsequent fast air cooling and by the strain-hardening effects of roll breakering and resultant age hardening of the steel at room temperature following this processing. This increase in hardness renders the steel unsuited for subsequent processing, but most particularly where the end product is processed directly from the hot-rolled and descaled strip.

It is an object of the present invention to provide a method of dry descaling of strip steel which is simpler and less expensive than those practiced in the prior art and one in which the forming characteristics of the steel are not adversely affected when applied to commercial quality and most drawing quality forming applications in the hot-rolled condition.

Steel strip for drawing purposes is usually coiled at a temperature of from 1350°-1400°F involving air cool on the run-out table. This practice accounts for a thick, tenacious scale that must be removed before being drawn or before cold reduction and annealing to lighter gauge drawing applications.

The scale that is formed is magnetite which is difficult to remove. This scale can be converted, when heated above 1076°F to wustite that is more easily removed. The wustite, however, is unstable and will revert to magnetite as the steel is cooled if special precautions are not used. It is also known that wustite forms a smooth interface with the iron base whereas the magnetite appears to have finger-like projections that extend between the grain boundaries of the underlying iron, making total clean-up difficult by any descaling method.

The equipment required to practice the present invention is a strip heating furnace of conventional type in which a strip can be heated to 1700°F in an atmosphere of products of combustion. In addition, there is required some mechanical means for removing scale such as brushes or shotblasting apparatus.

In practicing the invention, hot-rolled strip with a scale on its surface, usually magnetite, is continuously passed through a fuel fired or electric furnace having an atmosphere that can be ordinary hot products of combustion or air. The most efficient heating is obtained, regardless of fuel, when the products of combustion are neutral, but for purposes of the invention they can be slightly oxidizing or reducing. The furnace is maintained at such a temperature, and the strip is moved therethrough at such a speed the strip will be heated to a temperature of approximately 1700°F when it leaves the furnace. During the heating the magnetite scale is converted to wustite. As the scale converts it also increases microscopically in thickness, sufficient to oxidize below the finger-like projections of the magnetite, thus creating a substantially smooth interface between the wustite and the underlying metal.

Immediately after heating, the strip is cooled by blowing jets of air against both sides of the strip to cool it below 600°F and preferably to ambient temperature. This rapid cooling avoids reconversion of wustite back to magnetite until the temperature is below that at which the reconversion takes place. Thus, the strip is covered with a coating of easily removed scale in the form of wustite.

The strip is then moved directly to and through abrading apparatus to remove the scale. Strip cleaned in this fashion shows a clean, bright and smooth surface, and is immediately ready for subsequent processing.

Normally, when hot-rolled strip is coiled hot, from 1350°-1400°F, the strip according to the invention, is heated to about 1700°F. If the hot-rolled strip is coiled at a lower temperature of from 1000°-1100°F, the scale converting heating can be done at a lower temperature, in the range 1500°-1550°F. In either event, however, the strip is heated to well above the lower critical temperature in order both to convert the scale and increase scale thickness sufficiently to obtain a smooth interface. The strip can, of course, be heated to a temperature above 1700°F if desired. This increase, however, does not make the scale any easier to remove.

Ordinarily, the strip will be moved continuously through the furnace, air quench and abrading apparatus. It will be obvious, however, that the process is the same if the strip is heated and quenched, then coiled, with the abrading being done at a later time just prior to being used.

If deflating of the strip is desired it can be passed through a set of leveling rollers after the quench. Such

rollers will have no appreciable effect on the characteristics of the strip, but will tend to crack the scale and thus facilitate its removal.

While in accordance with the provisions of the States I have illustrated and described the best form of embodiment of my invention now known to me, it will be apparent to those skilled in the art that changes may be made in the form of the apparatus disclosed without departing from the spirit and scope of the invention set forth in the appended claims, and that in some cases certain features of my invention may be used to advantage without a corresponding use of other features.

What is claimed is:

1. The method of descaling a hot-rolled steel strip having a layer of magnetite on its surface which comprises heating the strip in a furnace in an normal fur-

nace atmosphere to a temperature of at least 1500° F thereby to convert the magnetite to wustite and increase the thickness thereof, immediately thereafter quenching the strip to below 600°F by directing air jets against both sides thereof at a rapid enough rate to prevent reconversion of the wustite to magnetite, and subsequently removing the wustite scale from the surface of the strip by abrasion.

10 2. The method of claim 1 in which the strip is heated to a temperature of approximately 1700°F.

15 3. The method of claim 1 in which heating of the strip is continued to increase the scale in thickness sufficiently to produce a substantially smooth interface between the scale and the underlying metal.

\* \* \* \* \*

20

25

30

35

40

45

50

55

60

65